

Dec. 29, 1931.

W. STUTLER

1,838,718

RECLAIMING SPENT OIL

Filed Dec. 13, 1929



## UNITED STATES PATENT OFFICE

WARNER STUTLER, OF BENNING ROAD AND DISTRICT LINE, DISTRICT OF COLUMBIA,  
ASSIGNOR TO WARNER STUTLER COMPANY, INC., OF WASHINGTON, DISTRICT OF  
COLUMBIA, A CORPORATION OF THE DISTRICT OF COLUMBIA

## RECLAIMING SPENT OIL

Application filed December 13, 1929. Serial No. 418,899.

This invention relates to a process of reclaiming spent lubricating oil, such as used oil from internal combustion engines.

The principal object of this invention is 5 to provide a simple, efficient and economical process whereby spent or used lubricating oil, such as that which is drained from the crank case of an automobile after it has become unsuited for further use may be purified, cleansed, and converted into a utilizable product.

Other objects and advantages of the invention will become apparent during the course of the following description.

15 Reclaiming of used lubricating oil has for a number of years attracted the attention of many persons, and many methods have been devised in an attempt to remove from used oils deleterious substances such as gasoline fractions which reduce the viscosity of the oil, solid suspended matter which due to its abrasive action renders the oil unsuitable for lubricating purposes, and acid forming substances such as water. However the re- 20 claimed oils produced by these processes have not proved thoroughly satisfactory.

I have discovered that if used oils are first clarified and subsequently distilled with agitation a materially improved character of 30 product is obtained. Such process includes the primary treatment of the used oil with water together with a clarifying agent, and the subsequent fractional distillation of the thus clarified product either without further 35 treatment or in conjunction with a bleaching agent as hereinafter described.

In the preferred practice of this invention a substantially large quantity of used or spent lubricating oil for instance, approximately 300 gallons, is mixed with approximately from 30 to 75 gallons of water and steam is passed through the body of such mixture until the temperature thereof is raised approximately to the boiling point of 45 water which condition is evidenced by the appearance of steam coming off from the top of the oil under treatment. Such temperature having been reached a clarifying agent is added to the material to precipitate 50 the impurities therein. Numerous clarify-

ing agents may be employed in the practice of my process but I prefer to employ a clarifying agent which is alkaline in nature. For example, soda ash, tri-sodium phosphate, a water-softening soap or soap powder. If 55 desired mixtures of such materials may be employed as will be apparent. However, I prefer to employ commercial soda ash. The amount of clarifying agent employed depends on the condition of the oil being treated but I have found that from 50 to 100 pounds of the clarifying agent will treat satisfactorily approximately 300 gallons of oil. When, as in the preferred embodiment 60 of the invention, commercial soda ash is used I have found that best results are obtained if approximately 75 pounds of this material are used to treat 300 gallons of oil.

In the actual practice of the process the used oil and water are mixed in any suitable 70 container and steam under a pressure of approximately 80 pounds per square inch is introduced into the mixture, preferably adjacent the bottom of the container. By this procedure the steam acts not only to heat 75 up the mass but at the same time serves to agitate it whereby the use of agitators is avoided, as would be required if the container were externally heated. After the mass has been heated until the steam begins 80 to rise from the top of the liquid the clarifying agent is added and the resulting mass is heated to a temperature of approximately from 225° to 300° F. when the steam is cut off. The mass is then allowed to stand until 85 the clarifying agent has caused the precipitation or settling of substantially all of the solid content in the oil. This is accomplished by the adhering of the clarifying agent to the fine particles of solid matter 90 whereby these particles settle relatively rapidly and do not remain in suspension as would, to a great extent, be the case if the clarifying agent were not employed. In the preferred practice the heated mass is permitted to stand overnight although in some instances standing for 5 hours is sufficient.

The thus clarified oil is drawn off and introduced into a still or similar apparatus 95 where it is heated in the manner hereinafter 100

described to drive off the lighter fractions of the oil and regulate the viscosity of the final product. Broadly speaking, the oil is heated in the still for approximately from 5 to two hours to three hours at a temperature of approximately from 500° to 650° F. and after the temperature of the oil has reached approximately 300° F. it is preferable to introduce steam into the lower portion of the still 10 and continue its introduction during the heat treatment. In conducting the heat treatment it is important that care be taken to prevent any substantial cracking of the oil. The "light ends" and steam which are driven off during the distilling process are discharged from the still and passed through a condenser whereby the "light ends" may be recovered for use, particularly as a penetrating oil or fuel oil.

20 After repeated experiments I have found that materially improved operating conditions and a substantially improved product are obtained if the heat treatment is conducted in a relatively elongated, upright still 25 provided with agitating means arranged adjacent the lower portion thereof which are so designed as to provide a whirling or rotary motion of the oil around the central vertical axis of the still and at the same time 30 to provide a current of the oil which is upward adjacent the periphery of the still and downward toward the central portion of the still. While I do not undertake to advance any theory for the improved results which 35 are obtained by conducting the heat treatment in the specific manner described, tests are convincing that greatly improved results are obtained as a direct result of this treatment.

40 At the completion of the heat treatment the oil is drawn off from the still and is cooled, as by running it through cold pipes, after which the oil is in condition for re-use as a lubricating oil. The oil is unbleached 45 but this does not impair its lubricating qualities in any way. However, if a bleached oil is desired this may be readily accomplished by introducing a bleaching agent into the oil during the process. For example, a bleached 50 product may be obtained by adding a bleaching earth such as bentonite, "metalloid" or the like, to the partially purified oil prior to its introduction into the still, and passing the oil after heat treatment thereof through a 55 filter press to remove the solid particles of the bleaching earth and coloring matter associated therewith. The particular advantage of introducing the bleaching agent into 60 the oil prior to the distilling thereof is that a particularly intimate contact of the bleaching agent with the oil is provided by the agitation in the still. The bleaching agent may be used in varying amounts but I have found 65 that particularly advantageous results are ob-

tained by employing one pound of bleaching agent to each gallon of oil treated.

As indicated above, the viscosity of the final product may be regulated according to the time and temperature of the heat treatment of the partially purified oil in the still. This is important particularly in the treatment of oil intended for use as crank case oil for automobiles since motorists demand several grades of oil as regards to viscosity, such as "light", "medium" and "heavy" oil. Generally speaking, these three types of oil correspond to oils having an S. A. E. viscosity of 30, 40 and 50.

An S. A. E. 30 oil may be obtained in the practice of my process by conducting the heat treatment referred to above at a temperature of approximately 500° F. for approximately 2 hours. By heating the oil to approximately from 550° to 600° F. for about two and one-half hours an S. A. E. 40 oil is obtained. Treatment at from approximately 600° to 650° F. for about three hours results in the production of an S. A. E. 50 oil.

In the accompanying drawings, I have indicated one embodiment of apparatus suitable for use in the practice of my process. In the drawings,

Figure 1 is a diagrammatic flow sheet of the process.

Figure 2 is a detail elevation of a preferred form of still with the wall thereof partly broken away, and,

Figure 3 is a transverse section taken on line 3-3 of Figure 2.

In the practice of my process in the form of apparatus indicated in the accompanying drawings, spent or used oil to be treated is introduced into a clarifying and settling tank 1 as at the point 2. The required amount of water is introduced as at the point 3 into the tank 1 and the mixture of oil and water is heated in the manner described above with steam admitted as at 4 through a pipe (not shown) which preferably extends into the tank and terminates in an open-end or nozzle at a point adjacent the bottom of the tank. When the mixture of oil and water has been heated to the desired temperature, as indicated above, a clarifying agent is introduced into the tank 1 as at the point 5. When the mass in the tank 1 has been heated to the desired temperature the steam is cut off and the mass allowed to stand until the impurities have settled to the bottom of the tank.

When the clarifying and settling operation has been completed the settling are removed through a pipe 6 and the clarified and partially purified oil is conveyed from the tank 1 through a pipe 7 into a still 8 where the oil is heated in the manner described above in the presence of steam which is preferably introduced into the still as at 9. The vapors driven off from the still during the heat treatment are conducted through a pipe

10 to a condenser 11 where these vapors are condensed and recovered as a light oil. At the completion of the heat treatment, the oil remaining in the still is drawn off through a 5 pipe 12 and introduced into a cooler 13 from which the oil is discharged as at 14 after the cooling operation has been completed.

As stated above, it is sometimes desirable to produce a bleached or light colored oil and in such event a bleaching agent of the character referred to above is introduced as at 15 into the pipe 7 prior to the passage of the oil into the still 8. When the oil is treated in the still 8 in the presence of a 15 bleaching agent the vapors driven off are collected in the condenser 11 in the usual manner but instead of passing the final product through the pipe 12 into the cooler 13 as is the practice when no bleaching agent is employed, the oil and the bleaching agent associated therewith are withdrawn as at 16 and passed through a filter press 17 to remove the solid particles present, after which the light colored oil is withdrawn as at 18 for use 25 as desired.

As stated above, I have found that greatly improved results are obtained if the heat treatment is conducted in a relatively elongated, upright still provided with agitating means arranged adjacent the lower portion thereof which are so designed as to provide a whirling or rotary motion of the oil around the central vertical axis of the still and at the same time to provide a current of the oil which is upward adjacent the periphery of the still and downward toward the central portion of the still. In Figures 2 and 3 of the drawings I have illustrated a type of still which is particularly adapted for use in the practice of my process. This still is designated generally by the reference numeral 20 and comprises an elongated cylinder closed at both ends. The agitation of the oil in the cylinder is affected primarily by means of a propeller 21. During the heating and agitating of the oil steam is admitted through a pipe and steam coil 22. The still is heated in any suitable manner but preferably by means of an oil burner, designated generally by the reference numeral 23, arranged in the fire-box 32.

The rotation of the propeller 21 is effected by means of a shaft 24 to the upper end of which is secured a bevel gear 25 meshing with a suitable gear 26 carried by the shaft 27 which is driven by any suitable source of power (not shown). The shaft 24 is carried in bearings 28 and 29 arranged in the upper and lower walls 30 and 31. The propeller 21 preferably consists of blades 33, 34, 35, and 36 which are so designed as to provide a whirling motion of the oil around the shaft 24 and also to provide an upward and downward current of oil in the manner described above and as indicated by the arrow in Fig-

ure 2. The vapors driven off from the oil during the heat treatment are discharged through the pipe 37 provided with a valve 38.

The apparatus just described constitutes the preferred form of apparatus to be used 70 in the practice of my process but it is to be understood that other forms of apparatus may be used if desired.

Whether the process is conducted so as to provide either a bleached or an unbleached 75 product, the oil produced will be found to be wholly satisfactory for reuse as a lubricant. In some instances, the oil will be found to be superior to the original oil due to the removal of impurities, such as certain 80 unsaturated compounds, which have been broken down by the heat of the engine lubricated by the original oil. Moreover, any impurities present which will react with the clarifying agent employed to form insoluble 85 compounds will be separated from the oil together with particles of carbon, dirt, metal particles and like solid impurities which serve to impair the lubricating properties of the oil. Moreover, any water present in the 90 oil treated will be driven off and a high-grade oil of the desired viscosity will be produced.

While I have described in detail the preferred practice of my process and a preferred 95 form of apparatus to be used, it is to be understood that the details of procedure and the form of apparatus may be variously modified without departing from the spirit of the invention or the scope of the subjoined claims. 100

I claim:

1. The herein described process of reclaiming spent lubricating oil which comprises heating the oil in the presence of water and an alkaline clarifying agent to a temperature of approximately from 225° to 300° F., permitting the resulting mass to stand to effect clarification of the oil, distilling the oil in the presence of steam and a bleaching agent while agitating the oil to drive off relatively low boiling hydrocarbons and to effect intimate contact between the oil and bleaching agent, and filtering the resulting oil to remove therefrom the bleaching agent and associated coloring matter. 105

2. The herein described process of reclaiming spent lubricating oil which comprises heating the oil in the presence of water and a clarifying agent, permitting the mass to stand to effect clarification of the oil, distilling the oil in the presence of steam in an upright column and agitating the oil in such manner that a whirling motion of the oil is secured and a current of oil is provided which is upward adjacent the outer portion of the column and downward adjacent the central vertical axis of the column, and cooling the resulting oil which has been substantially freed from light ends present in the oil by the distilling operation. 110

3. The herein described process of reclaiming spent lubricating oil which comprises heating the oil in the presence of water and a clarifying agent, permitting the mass to stand to effect clarification of the oil, distilling the oil in the presence of steam and a bleaching earth in an upright column, the steam being introduced adjacent the lower portion of said column, while agitating the oil in such manner that a whirling motion of the oil is secured and a current of oil is provided which is upward adjacent the outer portion of the column and downward adjacent the central vertical axis of the column, and filtering the resulting oil which has been substantially freed from light ends present by the distillation operation to remove therefrom the bleaching earth and associated coloring matter.
4. The herein described process of reclaiming spent lubricating oil which comprises heating and agitating the oil in the presence of water by means of a current of steam under pressure, adding soda ash to the mass, and heating the resulting mass to a temperature of approximately from 225° to 300° F., permitting the resulting mass to stand to effect clarification thereof, heating the resulting oil in the presence of steam and a bleaching earth in an upright column at a temperature of approximately from 500° to 650° F. for approximately from 2 to 3 hours, while agitating the oil in such manner that a whirling motion of the oil is secured and a current of oil is provided which is upward adjacent the outer portion of the column and downward adjacent the central vertical axis of the column, to drive off light ends present in the oil and simultaneously bleach the same, and passing the resulting oil through a filter press to remove solids therefrom.

In testimony whereof I affix my signature.  
WARNER STUTLER.

45

50

55

80